# EUROPEAN PATENT SPECIFICATION

(11) **EP 3 967 789 B1**
(45) Date of publication and mention of the grant of the patent: **13.08.2025**
(21) Application number: 20195838.6
(22) Date of filing: 11.09.2020
(51) Int. Cl.: B05B 1/06, B05B 1/14, B05B 9/03, B05B 16/00, C23G 3/02, C23G 1/08

(54) **ULTRAFAST PICKLING METHOD AND INSTALLATION THEREFOR**
ULTRASCHNELLES BEIZVERFAHREN UND ANLAGE DAFÜR
PROCÉDÉ DE DÉCAPAGE ULTRARAPIDE ET INSTALLATION ASSOCIÉE

(43) Date of publication of application: 16.03.2022
(73) Proprietor: Centre de Recherches Métallurgiques ASBL - Centrum voor Research in de Metallurgie VZW, 1000 Bruxelles (BE)
(72) Inventor: FLAMENT, Sébastien, 4530 VIEUX WALEFFE (BE); UIJTDEBROEKS, Hugo, 3500 HASSELT (BE); TUSSET, Victor, 4680 OUPEYE (BE); NOVILLE, Jean-François, 4041 MILMORT (BE); SMAL, Julien, 4000 ROCOURT (BE)
(74) Representative: AWA Benelux

(56) References cited:
- EP-A1- 3 453 465
- EP-A2- 1 008 676
- WO-A1-2020/217180
- US-A- 4 270 317
- US-A- 6 016 819

## Description

### Field of the Invention

The present invention relates to a fast method for the pickling of a steel product in a continuous manufacturing line. The invention also relates to the installation for performing the method.

### Background and Prior Art

In the steel industry, many processes that occur at high temperature leave an oxide layer or scale on the product surface. In particular, prior to cold rolling operation, hot rolled steel has to be passed through a pickling line so as to remove the scale from its surface. Presently pickling is more and more the bottleneck process when coupled to the cold rolling mill (Pickling Line Tandem Cold Mill - PLTCM).

Several acid pickling media have been used depending on the specific product to pickle (sulfuric, hydrochloric, hydrofluoric, nitric acids, etc.). However acid pickling of carbon steel is usually limited to pickling with a hydrochloric solution.

Nowadays, steels are more and more alloyed, especially with silicon and manganese. Steels containing silicon are especially prone to the formation of fayalite (orthorhombic iron silicate Fe₂SiO₄) during reheating of the slab. Fayalite becomes liquid above 1173°C, which is always the case in reheating furnaces (T>1200°C). This liquid phase infiltrates the oxide down to the steel-oxide interface and "sticks" to the metal. Fayalite is difficult to remove during hydraulic descaling (hot rolling process). In particular, when present at the entry of the pickling line, Fayalite is very difficult to be removed by the HCl pickling liquor because of its low solubility.

When such products enter the pickling line, the strip speed has to be reduced in order to ensure a certain pickling time necessary to remove the oxide layer. In the worst cases very low pickling speeds are even not sufficient to remove all the oxides and specifically fayalite from the steel surface.

Pickling of a steel strip is a chemical process based on the dissolution of oxides in acid (with HCl concentration usually between 30 and 180 g/l) at a temperature up to 80°C. Oxide dissolution increases with acid concentration, temperature and turbulence of the pickling liquor :
- acid concentration is managed by a cascade of tanks containing pickling media from a last tank to a first one of the line. Fresh acid (180 g/l) is fed in the last pickling tank, with liquid in countercurrent circulation in respect of solid product ;
- as a temperature of 80°C is usually the maximum temperature used in HCl pickling process, temperature can hardly be increased well above when using polypropylene (PP) for manufacturing the tanks, which equips more and more lines ;
- increasing turbulence is precisely the purpose of the present patent application : increasing turbulence to refresh more rapidly the free acid in the electric double layer directly increases the pickling process efficiency.

Several pickling methods are known in the art for removing scale :
- deep tank pickling : the steel strip is dipped in acid solution in deep working tanks and with a large catenary size only supported by inlet and outlet skids. The acid solution presents extremely slow flow motion ;
- shallow tank pickling : the size of steel strip catenary is reduced as well as the depth of acid fluid. The acid fluid circulates largely with the steel strip inside the tank and the relative flow rate between the strip and the acid fluid is small, causing limitation to increase pickling speed ;
- in Turboflo^{™} pickling lines developed by Danieli, US (WO 00/71267 A1), where pickling tanks are divided in a number of cells, the descaling process is accelerated thanks to turbulence created by sprays at the entry, the exit and at the sides and by changes of the cell section of the channel ;

- in US 5,545,260 A (SMS), turbulence is created by high pressure (3 bar) spray headers located at the inlet and at the outlet of the tank ;
- in EP 3 029 164 B1 (CMI UVK GmbH), there is combination of a spraying tank (P < 3bar, spray headers located every 40-50 cm) in cascade with an immersion tank. Speed is increased with turbulence ;
- in the iBox pickling tank of Primetals, the acid solution is circulated by strip running effect and continuously heated up by internal heat exchangers. External circulation system and heat exchanger are not required and as a result, iBox pickling tank has the benefits of low maintenance and radiation losses, low clogging risk as well as rapid heating up. However turbulence is only controlled by strip velocity ;
- as an alternative to acid pickling, in the EPS technology (Eco pickled surface, The Material Works, see e.g. US 8, 066,549 B2), slurry blasts are propelled on the strip in uniform streams. Slurry blasting is a wet abrasive blasting process that combines a fine-particle metallic abrasive with a carrier liquid, most commonly water. The slurry mixture is fed into a rotating impeller which propels it at high velocity across the object to be cleaned. Its advantages are to be well suited for processing a large product mix on the same line (carbon steel, stainless steel, alloyed steel, etc.), no overpickling, to provide a rust resistant surface without oiling and a more homogeneous surface aspect. However that is a slow process, with higher roughness and need for slurry blasts regeneration.

Highly turbulent technologies which are further investigated in this application have been considered for a long time for cooling purposes. As a matter of fact, since the 1980's, the Applicant has studied the opportunity to apply cooling technologies with very high cooling power (up to 5 MW/m²), firstly for high-strength plates and secondly for rolling mill rolls, which are alternative to conventional cooling technologies (see e.g. H. Uijtdebroeks et al., High turbulence roll cooling, European Commission, contract No 7215-PP/075, 2002-2005, Final report EUR 22972). As such a very high cooling power cannot be obtained by normal laminar jet nozzles, high turbulence cooling technologies were investigated. Cooling heads have been designed to operate on the one side in so-called "high turbulence low pressure regime" (HTLP) and on the other side in so-called "water pillow cooling" (WPC). The distance between the header and the plate, strip or roll determines whether the dominant cooling effect will be obtained through either WPC or HTLP or a combination of both. HTLP requires a much smaller plate, strip or roll/header gap distance compared to WPC. The smaller gap creates a higher degree of turbulence. Therefore it results in a significant increase in thermal exchange.

In HTLP cooling, the cooling header is located at close distance of the strip, plate or roll surface, typically 3-4 mm. The electrolyte, e.g. water or water solution, is injected in a central gap and forced to flow between the roll or strip surface and the cooling module. The pursued principle is also to create a high turbulence in the gap between the surface and the header so as to increase thermal exchange between the surface and the cooling liquid.

The WPC cooling has been developed to perform selective cooling of long and flat products having a high heat transfer coefficient. The WPC cooling device is placed at short distance, typically of 10 to 100 mm from the surface to cool. Owing to this close distance and thanks to water projection, a water cushion is formed between the module and the surface. Injection of straight water jets through holes drilled in the header maintains the cushion while creating high turbulence therein. The particularity is that high heat transfer coefficients are obtained at low pressure. With WPC a very homogeneous cooling pattern is obtained over the whole surface to cool. This homogeneity is related to the number of straight water jets in the header, the cooling pattern and the applied pressure. The required operating pressure typically varies from 2 to 5 bar. The thickness of the water cushion varies from 10 to 100mm.

The cooling efficiency is strongly influenced by the total amount of water injected. The performance increases with the increase of water flow, if necessary combined with side guides. For the same heat flux during cooling a lower flow rate and pressure are required compared to the traditional flat jet spray cooling configurations.

The Applicant has obtained efficient cooling of the work rolls in flat and long product mills thanks to the application of a breakthrough technology called "High Turbulence Roll Cooling" (HTRC) (patented under EP 2 114 584 B1). In this concept, a turbulent water cushion is formed around the work roll surface with a controlled and forced water circulation. This technology has continuously been improved over the last years. Besides the possibility to control the distance between the cooling header and the work roll surface ( position-controlled HTRC), the turbulence of the water is created combining the water pillow cushion technology and the high turbulent low pressure cooling principle. For a similar flow rate, the heat transfer coefficient is increased by 25% compared to the first generation of HTRC and by more than the double compared to a traditional roll cooling system with flat jet nozzles operating up to 15 bar. As the enhanced HTRC unit operates at a low pressure (2 to 3 bar), the energy saving reaches values close to 85 to 90% compared to a conventional cooling system.

Document US 4,270,317 A discloses an apparatus used in the treatment of a sheet of metal, in which the sheet of metal is guided in a horizontal pathway between successive treatment tanks or units having horizontally elongated chambers with two rows of oppositely disposed and horizontally aligned nozzles between which the sheet of metal travels on a liquid bed that is created by the nozzles which are designed to direct streams of liquid, under pressure, against the traveling metal sheet at angles that are substantially less than 90° relative to the plane in which the metal sheet travels. A unique liquid seal and conventional blowoff device are utilized at each opening through which the traveling metal sheet enters and exits the various chambers, as a means of maintaining the liquid within the chamber and preventing it from being carried away by the traveling metal sheet into an adjacent chamber where the appearance of such liquid may have a deleterious effect upon the process being carried out in that particular chamber. The individual units are also free of brushes and other such devices which are normally used to aid in the cleaning of the sheet of metal.

Document EP 1 008 676 A2 discloses a process and a device for the continuous pickling in a non-oxidizing acid bath of hot-rolled steel strips, characterised in that the strip is subject to the pickling action of the bath, additioned of a pickling catalyst, under turbulent conditions. This device comprises the following in combination : a closed storage tank containing the catalyst-additioned pickling bath; at least one cell, located above the free surface of the pickling bath, inside which the strip to be pickled, possibly guided by supporting rolls, travels horizontally ; immersed nozzles, provided above and below the strip, located and shaped so as to feed under pressure the pickling bath to the cell, to create a directional flow of the pickling bath itself that generates the required turbulent conditions ; means for drawing the pickling bath from the tank and delivering it to the nozzles ; and means for recirculating the pickling bath from the cell to the tank.

Document WO 2020/217180 A1 concerns a continuous pickling process and plant for the treatment of metal products in the form of a strip or tube. The device includes a plurality of acid solution process tanks each divided into a plurality of turbulence cells and a recirculation system of the acid solution. The plant also includes, upstream of the plurality of process tanks, a device for heating the metal product, namely an induction heating system and/or a tunnel with water sprays. Devices are described to increase turbulence in the tanks and to accelerate pickling, e.g. by adding fresh acid in the first tank. The invention optimizes the effect of the acid and reduces the residence time of the strip in the plant.

### Aims of the Invention

The present invention aims to provide a pickling installation and method for manufacturing metal products such as steel strips with reduced pickling time, especially in presence of hard to remove oxides such as fayalite on the steel surface.

### Summary of the Invention

A first aspect of the present invention relates to a pickling installation for applying a pickling treatment to a steel strip (10) in continuous movement, said pickling treatment using an acid solution, said pickling installation comprising :
- a plurality of cascading treatment tanks among which at least one treatment tank comprising a spray/injection section for spraying/injecting the acid solution on the metal strip, and
- collection means for retrieving the sprayed acid solution and redirect the same to each spray/injection section ;
the at least one treatment tank comprising a first header in use in front of a first face of the metal strip and a second header in use in front of a second face of the metal strip, wherein :
- in a first treatment tank configuration, each of the first header and the second header have an internal flat surface intended to be parallel respectively to the first and second faces of the metal strip, and at a distance thereof, defining a first gap and a second gap respectively, said first header and said second header comprising each a plurality of holes drilled through the internal flat surface according to a defined 2D-pattern, for spraying the acid solution to the metal strip in straight jets, under conditions suitable to create in use at the surface of the metal strip a highly turbulent liquid cushion, or alternately ;
- in a second treatment tank configuration, each of the first header and the second header have an internal flat surface intended to be parallel respectively to the first and second faces of the metal strip, and at a distance thereof, defining a first gap and a second gap respectively, acid solution injection means being provided at an edge injection opening of each respective gap, under conditions suitable to create in use at the surface of the metal strip a highly turbulent liquid zone occupying the whole gap volume, or alternately ;
- a third treatment tank configuration combines the first treatment tank configuration and the second treatment tank configuration ;
and wherein, either in the first treatment tank configuration (1A) or in the second treatment tank configuration (1B), said internal flat surface (6), except at the locations of the holes drilled therein in case of the first configuration (1A), is continuous.

According to particular embodiments, the pickling installation further comprises at least one of the following characteristics or a suitable combination thereof :
- the acid solution used contains abrasive particles ;
- the collection means comprise at least one storage tank and at least one pump as well as means for injecting fresh acid into the pickling tanks in counter-current in respect of the cascading direction ;
- the pickling installation comprises at least one other treatment tank ;
- the at least one other treatment tank is an immersion or a rinsing treatment tank ;
- lateral side guides are provided for maintaining the liquid cushion or the highly turbulent zone in the gap or the first and the second gaps are designed to form a tunnel having a width equal to the width of the line ;
- the at least one pump is made of a material able to resist to abrasive particles present inside the acid solution, selected from the group consisting of ceramic, graphite, polyvinylidene fluoride (PVDF), and polytetrafluoroethylene (PTFE) ;
- the at least one pump is designed so that the abrasive particles are injected by venturi effect after a pump outlet ;
- the first gap and the second gap are different, in particular the first gap is greater than the second gap ;
- the injection means being provided at an edge injection opening of the gap are co-current or counter-current to the strip, in this last case to increase the relative speed between the strip and pickling flow.

A second aspect of the present invention relates to a method for applying a pickling treatment to a metal strip in continuous movement, using the pickling installation according to anyone of the preceding claims, wherein it comprises the steps of :
- providing the pickling installation with an acid solution ;
- directing the moving metal strip into at least one treatment tank comprising a spraying/injection section for spraying/injecting the acid solution on the metal strip, and spraying/injecting the acid solution on one or both faces of the metal strip under high turbulence conditions ;
- retrieving the acid solution sprayed on the metal strip and redirecting again the same to the spraying sections using the collection means.

According to particular embodiments, the pickling method further comprises at least one of the following characteristics or a suitable combination thereof :
- the metal strip is further directed to be treated in one or more other treatment tanks ;
- the metal strip is a steel strip, selected from the group consisting of a carbon steel strip, a stainless steel strip, and an alloyed steel strip ;
- the acid solution used is a hydrochloric acid, sulphuric acid, nitric acid, phosphoric acid or hydrofluoric acid solution ;
- acid insoluble abrasive mineral particles are added to the acid solution ;
- the Mohs hardness of the acid insoluble abrasive mineral particles is comprised between 4 and 7, and preferably is greater than or equal to 5 ;
- the acid insoluble abrasive mineral particles are selected from the group consisting of corundum, glass microballs, alumina, silicate, silicon carbide and zirconium ;
- the flow rate of the sprayed/injected acid solution is selected so as to obtain in the first tank configuration a thickness of the highly turbulent liquid cushion equal to the thickness of the gap ;
- the maximum temperature of the acid solution is about 80°C, for example in case of use of polypropylene, PVDF, PTFE tanks ;
- the abrasive particles are recovered at the end of the process, for example by filtration or decantation.

According to a particular embodiment, the metallurgical line and thus the continuous strip movement is horizontal. In this case, the first header, the second header respectively, is an upper header, respectively a lower header. Further the first face of the strip, the second face of the strip respectively, is an upper face, a lower face respectively.

According to another embodiment, the metallurgical line and thus the continuous strip movement is vertical.

### Brief Description of the Drawings

FIG. 1 is a schematic view representing a metallurgical pickling line according to prior art.
FIG. 2A is a schematic cross-sectional longitudinal view representing the principle of acid pickling under high turbulence WPC conditions applied to a moving metal strip.
FIG. 2B is a schematic cross-sectional longitudinal view representing the principle of acid pickling under high turbulence HTLP conditions applied to a moving metal strip.
FIG. 2C is a schematic cross-sectional longitudinal view representing the principle of acid pickling under high turbulence respective WPC and HTLP conditions applied to a moving metal strip.
FIG. 3 is a schematic cross-sectional longitudinal view representing the principle of acid pickling under high turbulence respective WPC and HTLP conditions applied to a moving metal strip, in presence of abrasive particles in the tank solution.

### Description of a Preferred Embodiments of the Invention

In the pickling method according to a first embodiment of the present invention, turbulence of the pickling solution is increased through the WPC and/or HTLP principles or a combination of both technologies.

Accordingly, as schematically represented in FIG. 2A, a WPC highly turbulent regime is applied to the acid solution present in one or more tanks of the pickling installation.

Let us consider the pickling process of a metal strip 10, such as a steel strip, in horizontal processing. The method could also be applicable to long products. The pickling installation comprises a number N of tanks into which the metal strip 10 moves successively on rolls (not represented). Each (or at least one) tank 1A comprises an upper header 2A in front of the upper face of the strip and a lower header 2B in front of the lower face of the strip. Each header 2A, 2B comprises holes 3 drilled in the header 2A, 2B through which injection of straight water jets 4 is performed at high flow rate so as to maintain a liquid cushion 5' in the respective upper gap 5A and lower gap 5B between the headers 2A, 2B and the strip, with high turbulence therein. The jets are straight jets and not flared jets such as those obtained with ordinary flat nozzles. The height of the liquid cushion 5', typically 10-100mm, can be lower than the distance 5A, 5B separating the internal header surface 6 and the strip 10.

When using WPC, pressure will be in the range 1 to 5 bars and the specific flow rate in the range of 10 to 150 m³/h/m² of surface.

Alternatively, as schematically represented in FIG. 2B, a HTLP highly turbulent regime is applied to the acid solution present in (a) tank(s) 1B of the pickling installation. FIG. 2C shows an embodiment with the combined use of both principles cites here above. In this case, the internal header surface 6 is located very close to the strip (typically 2-5 mm) and the electrolyte is forced to enter the gap 5A, 5B between the header plate 6 and the strip 10, through one opening 7 located at one side of the device, creating thereby a highly turbulent zone.

When HTLP is used, pressure will be in the range of 0.5 to 2 bars and the specific flow rate per side in the range of 50 to 120 m³/h/m of width.

Note that, for either WPC or HTLP, the value of the pressure obtained is linked to the specific flow rate by the design of the nozzles or injector.

In a second embodiment, beside the chemical action of acid and in addition of it, in order to further and efficiently assist in the removal of hard to dissolve oxides like fayalite, the inventors further assert that a mechanical action would help for strengthening removal of this kind of oxide. Such a mechanical action is intended under the form of an addition of abrasive particles 20 propelled on the strip surface in a highly turbulent tank (FIG. 3) so as to further decrease the pickling time.

Preferably, abrasive particles 20 non-soluble in acid, such as corundum, glass microballs, alumina, silicate, silicon carbide, zirconium, etc., will be used. The Mohs hardness of the acid insoluble abrasive mineral particles 20 will be comprised between 4 and 7, and preferably will be higher or equal to 5. Particles with Mohs hardness of 5 minimum have excellent resistance to HCl at all useful concentrations and temperatures.

In this case, an innovation consists in using a double action made of a chemical action and a mechanical action respectively due to acid and abrasive particles to optimize the reduction of pickling time.

So the materials used in the pickling installation will be suitably chosen so as to resist to the pickling media, acid and abrasive particles.

Advantageously, the abrasive particles will be recovered at the end of the process for example by filtration or decantation.

FIG. 3 schematically represents the principle of acid pickling under high turbulence with respective WPC and HTLP conditions, as described above, applied to a moving metal strip, but now in additional presence of abrasive particles in the tank solution.

### Reference symbols

- 1A: WPC acid pickling tank
- 1B: HTLP acid pickling tank
- 1C: WPC and HTLP acid pickling tank
- 1D: WPC acid pickling tank with abrasive particles
- 1E: HTLP acid pickling tank with abrasive particles
- 1F: WPC and HTLP acid pickling tank with abrasive particles
- 2A, 2B: Upper header, lower header (horizontal processing)
- 3: Hole drilled in header (WPC)
- 4: Straight jet (WPC)
- 5A, 5B: Upper gap, lower gap (horizontal processing)
- 5': Liquid cushion
- 6: Header internal flat surface
- 7: Injection opening (HTLP)
- 8: Acid solution tank
- 9: Pump
- 10: Metal strip
- 11, 12, 13,: Pickling treatment tank
- 18: Injection line for fresh acid
- 20: Abrasive mineral particle

## Claims

1. A pickling installation for applying a pickling treatment to a metal strip (10) in continuous movement, said pickling treatment using an acid solution, said pickling installation comprising :
- a plurality of cascading treatment tanks (1A, 1B, 1C, 1D, 1E, 1F, 11, 12, 13, etc.) among which at least one treatment tank (1A, 1B, 1C) comprising a spray/injection section (3, 4, 7) for spraying/injecting the acid solution on the metal strip (10), and
- collection means (8, 9) for retrieving the sprayed acid solution after use and redirect the same to each spray/injection section (3, 4, 7) ;
the at least one treatment tank (1A, 1B, 1C) comprising a first header (2A) in use in front of a first face of the metal strip (10) and a second header (2B) in use in front of a second face of the metal strip (10), wherein
- in a first treatment tank configuration (1A), each of the first header (2A) and the second header (2B) have an internal flat surface (6) intended to be parallel respectively to the first and second faces of metal strip (10), and at a distance thereof, defining a first gap (5A) and a second gap (5B) respectively, said first header (2A) and said second header (2B) comprising each a plurality of holes (3) drilled through the internal flat surface (6) according to a defined 2D-pattern, for spraying the acid solution to the metal strip (10) in straight jets (4), under conditions suitable to create in use at the surface of the metal strip (10) a highly turbulent liquid cushion (5'), or alternately
- in a second treatment tank configuration (1B), each of the first header (2A) and the second header (2B) have an internal flat surface (6) intended to be parallel respectively to the first and second faces of the metal strip (10), and at a distance thereof, defining a first gap (5A) and a second gap (5B) respectively, acid solution injection means being provided at an edge injection opening (7) of each respective gap (5A, 5B), under conditions suitable to create in use at the surface of the metal strip (10) a highly turbulent liquid zone occupying the whole respective gap (5A, 5B) volume, or alternately
- a third treatment tank configuration (1C) combines the first treatment tank configuration (1A) and the second treatment tank configuration (1B) ;
and wherein, either in the first treatment tank configuration (1A) or in the second treatment tank configuration (1B), said internal flat surface (6), except at the locations of the holes drilled therein in case of the first treatment tank configuration (1A), is continuous.

2. The pickling installation according to claim 1, wherein the acid solution used contains abrasive particles.

3. The pickling installation according to claim 1 or 2, wherein the collection means (8, 9) comprise at least one storage tank (8) and at least one pump (9) as well as means (18) for injecting fresh acid into the pickling tanks in counter-current in respect of the cascading direction.

4. The pickling installation according to claim 1 or 2, wherein it comprises at least one other treatment tank (11, 12, 13, ...).

5. The pickling installation according to claim 4, wherein the at least one other treatment tank (11, 12, 13, ...) is an immersion or a rinsing treatment tank.

6. The pickling installation according to claim 1 or 2, wherein lateral side guides are provided for maintaining the liquid cushion (5') or the highly turbulent zone in the gap (5A, 5B) or wherein the first and the second gaps (5A, 5B) are designed to form a tunnel having a width equal to the width of the line.

7. The pickling installation according to claim 3, wherein the at least one pump (9) is made of a material able to resist to abrasive particles present inside the acid solution, selected from the group consisting of ceramic, graphite, polyvinylidene fluoride (PVDF), and polytetrafluoroethylene (PTFE).

8. The pickling installation according to claim 3, wherein the at least one pump (9) is designed so that the abrasive particles are injected by venturi effect after a pump outlet.

9. The pickling installation according to claim 1 or 2, wherein the first gap (5A) and the second gap (5B) are different.

10. The pickling installation according to claim 1 or 2, wherein the injection means being provided at an edge injection opening (7) of the gap (5A, 5B) are co-current or counter-current to the strip, in this last case to increase the relative speed between the strip and pickling flow.

11. A method for applying a pickling treatment to a metal strip (10) in continuous movement, using the pickling installation according to anyone of the preceding claims, wherein it comprises the steps of :
- providing the pickling installation with an acid solution ;
- directing the moving metal strip (10) into at least one treatment tank (1A, 1B, 1C) comprising a spray/injection section (3, 4, 7) for spraying/injecting the acid solution on one or both faces of the metal strip (10) under high turbulence conditions ;
- retrieving the acid solution sprayed on the metal strip (10) and redirecting again the same to the spray/injection sections (3, 4, 7) using the collection means (8, 9).

12. The pickling method according to claim 11, wherein the metal strip (10) is further directed to be treated in one or more other treatment tanks (11, 12, 13, ...).

13. The pickling method according to claim 11, wherein the metal strip (10) is a steel strip selected from the group consisting of a carbon steel strip, a stainless steel strip and an alloyed steel strip.

14. The pickling method according to claim 11, wherein the acid solution used is a hydrochloric acid, sulphuric acid, nitric acid, phosphoric acid or hydrofluoric acid solution.

15. The pickling method according to claim 11, wherein acid insoluble abrasive mineral particles (20) insoluble in acid are added to the acid solution.

16. The pickling method according to claim 15, wherein the Mohs hardness of the acid insoluble abrasive mineral particles (20) is comprised between 4 and 7.

17. The pickling method according to claim 15, wherein the acid insoluble abrasive mineral particles (20) are selected from the group consisting of corundum, glass microballs, alumina, silicate, silicon carbide and zirconium.

18. The pickling method according to claim 11, wherein the flow rate of the sprayed/injected acid solution is selected so as to obtain in the first tank configuration (1A) a thickness of the highly turbulent liquid cushion (5') equal to the thickness of the gap (5).

19. The pickling method according to claim 11, wherein the maximum temperature of the acid solution is 80°C, in case of use of polypropylene, PVDF, PTFE tanks.

20. The pickling method according to claim 11, wherein the abrasive particles are recovered at the end of the process, by filtration or decantation.

## Patentansprüche

1. Beizanlage zum Anwenden einer Beizbehandlung auf ein Metallband (10) in kontinuierlicher Bewegung, wobei die Beizbehandlung eine Säurelösung verwendet, die Beizanlage umfassend:
- eine Vielzahl von kaskadierenden Behandlungsbehältern (1A, 1B, 1C, 1D, 1E, 1F, 11, 12, 13 usw.), wovon denen mindestens ein Behandlungsbehälter (1A, 1B, 1C) einen Sprüh-/Einspritzabschnitt (3, 4, 7) zum Sprühen/Einspritzen der Säurelösung auf das Metallband (10) umfasst, und
- Auffangeinrichtungen (8, 9), um die gesprühte Säurelösung nach Gebrauch aufzufangen und sie zurück zu dem jeweiligen Sprüh-/Einspritzabschnitt (3, 4, 7) zu leiten;
der mindestens eine Behandlungsbehälter (1A, 1B, 1C) umfassend einen ersten Verteiler (2A), der vor einer ersten Seite des Metallbands (10) in Gebrauch ist, und einen zweiten Verteiler (2B), der vor einer zweiten Seite des Metallbands (10) in Gebrauch ist, wobei
- jeder von dem ersten Verteiler (2A) und dem zweiten Verteiler (2B) in einer ersten Behandlungsbehälterkonfiguration (1A) eine innere flache Oberfläche (6) aufweisen, die dazu bestimmt ist, parallel zu jeweils der ersten und der zweiten Fläche eines Metallbands (10) und in einem Abstand davon zu sein und jeweils einen ersten Spalt (5A) und einen zweiten Spalt (5B) zu definieren, der erste Verteiler (2A) und der zweite Verteiler (2B) jeweils umfassend eine Vielzahl von Löchern (3), die gemäß einem definierten 2D-Muster durch die innere flache Oberfläche (6) gebohrt sind, um die Säurelösung unter Bedingungen, die geeignet sind, um im Gebrauch an der Oberfläche des Metallbands (10) ein hochturbulentes Flüssigkeitskissen (5') zu erzeugen, in geraden Strahlen (4) auf das Metallband (10) zu sprühen, oder alternativ
- jeder von dem ersten Verteiler (2A) und dem zweiten Verteiler (2B) in einer zweiten Behandlungsbehälterkonfiguration (1B) eine innere flache Oberfläche (6) aufweisen, die dazu bestimmt ist, parallel zu jeweils der ersten und der zweiten Fläche des Metallbands (10) und in einem Abstand davon zu sein und jeweils einen ersten Spalt (5A) und einen zweiten Spalt (5B) zu definieren, wobei Säurelösungseinspritzeinrichtungen an einer Randeinspritzöffnung (7) jedes jeweiligen Spalts (5A, 5B), unter Bedingungen bereitgestellt sind, die geeignet sind, um im Gebrauch an der Oberfläche des Metallbands (10) eine hochturbulente Flüssigkeitszone zu erzeugen, die das gesamte Volumen des jeweiligen Spalts (5A, 5B) einnimmt, oder alternativ
- wobei eine dritte Behandlungsbehälterkonfiguration (1C) die erste Behandlungsbehälterkonfiguration (1A) und die zweite Behandlungsbehälterkonfiguration (1B) kombiniert;
und wobei entweder in der ersten Behandlungsbehälterkonfiguration (1A) oder in der zweiten Behandlungsbehälterkonfiguration (1B) die innere flache Oberfläche (6), außer an den Stellen der darin gebohrten Löcher im Fall der ersten Behandlungsbehälterkonfiguration (1A), durchgehend ist.

2. Beizanlage nach Anspruch 1, wobei die verwendete Säurelösung abrasive Partikel enthält.

3. Beizanlage nach Anspruch 1 oder 2, wobei die Auffangeinrichtungen (8, 9) mindestens einen Speicherbehälter (8) und mindestens eine Pumpe (9) sowie Einrichtungen (18) zum Einspritzen von frischer Säure in die Beizbehältern im Gegenstrom in Bezug auf die Kaskadenrichtung umfassen.

4. Beizanlage nach Anspruch 1 oder 2, **dadurch gekennzeichnet, dass** sie mindestens einen weiteren Behandlungsbehälter (11, 12, 13, ...) umfasst.

5. Beizanlage nach Anspruch 4, wobei der mindestens eine weitere Behandlungsbehälter (11, 12, 13, ...) ein Tauch- oder Spülbehandlungsbehälter ist.

6. Beizanlage nach Anspruch 1 oder 2, wobei seitliche Seitenführungen bereitgestellt sind, um das Flüssigkeitskissen (5') oder die hochturbulente Zone in dem Spalt (5A, 5B) zu halten, oder wobei der erste und der zweite Spalt (5A, 5B) konstruiert sind, um einen Tunnel zu bilden, der eine Breite gleich wie die Breite der Leitung aufweist.

7. Beizanlage nach Anspruch 3, wobei die mindestens eine Pumpe (9) aus einem Material gefertigt ist, das in der Lage ist, den in der Säurelösung vorhandenen abrasiven Partikeln zu widerstehen, ausgewählt aus der Gruppe, bestehend aus Keramik, Grafit, Polyvinylidenfluorid (PVDF) und Polytetrafluorethylen (PTFE).

8. Beizanlage nach Anspruch 3, wobei die mindestens eine Pumpe (9) konstruiert ist, sodass die abrasiven Partikel durch Venturi-Effekt nach einem Pumpenauslass eingespritzt werden.

9. Beizanlage nach Anspruch 1 oder 2, wobei der erste Spalt (5A) und der zweite Spalt (5B) verschieden sind.

10. Beizanlage nach Anspruch 1 oder 2, wobei die Einspritzeinrichtungen, die an einer Randeinspritzöffnung (7) des Spalts (5A, 5B) bereitgestellt sind, im Gleichstrom oder im Gegenstrom zu dem Band sind, um im letzteren Fall die relative Geschwindigkeit zwischen dem Band und der Beizströmung zu erhöhen.

11. Verfahren zum Anwenden einer Beizbehandlung auf ein Metallband (10) in kontinuierlicher Bewegung unter Verwendung der Beizanlage nach einem der vorherigen Ansprüche, wobei es die folgenden Schritte umfasst:
- Bereitstellen einer Säurelösung an die Beizanlage;
- Lenken des sich bewegenden Metallbands (10) in mindestens einen Behandlungsbehälter (1A, 1B, 1C), umfassend einen Sprüh-/Einspritzabschnitt (3, 4, 7) zum Sprühen/Einspritzen der Säurelösung auf eine oder beide Seiten des Metallbands (10) unter hohen Turbulenzbedingungen;
- Abnehmen der auf das Metallband (10) gesprühten Säurelösung und deren erneutes Leiten zu den Sprüh-/Einspritzabschnitten (3, 4, 7) unter Verwendung der Auffangeinrichtungen (8, 9).

12. Beizverfahren nach Anspruch 11, wobei das Metallband (10) weitergelenkt wird, um in einem oder mehreren anderen Behandlungsbehälter (11, 12, 13, ...) behandelt zu werden.

13. Beizverfahren nach Anspruch 11, wobei das Metallband (10) ein Stahlband ist, das ausgewählt ist aus der Gruppe, bestehend aus einem Kohlenstoffstahlband, einem Edelstahlband und einem legierten Stahlband.

14. Beizverfahren nach Anspruch 11, wobei die verwendete Säurelösung eine Salzsäure-, Schwefelsäure-, Salpetersäure-, Phosphorsäure- oder Fluorwasserstoffsäurelösung ist.

15. Beizverfahren nach Anspruch 11, wobei zu der Säurelösung säureunlösliche abrasive mineralische Partikel (20) hinzugefügt werden, die in Säure unlöslich sind.

16. Beizverfahren nach Anspruch 15, wobei die Mohs-Härte der säureunlöslichen abrasiven mineralischen Partikel (20) zwischen 4 und 7 liegt.

17. Beizverfahren nach Anspruch 15, wobei die säureunlöslichen abrasiven mineralischen Partikel (20) ausgewählt sind aus der Gruppe, bestehend aus Korund, Glasmikrokugeln, Aluminiumoxid, Silikat, Siliziumkarbid und Zirkonium.

18. Beizverfahren nach Anspruch 11, wobei die Durchflussmenge der gesprühten/eingespritzten Säurelösung gewählt ist, um in der ersten Behälterkonfiguration (1A) eine Stärke des hochturbulenten Flüssigkeitskissens (5') zu erreichen, die der Stärke des Spalts (5) entspricht.

19. Beizverfahren nach Anspruch 11, wobei die Höchsttemperatur der Säurelösung bei Verwendung von Polypropylen-, PVDF- oder PTFE-Behältern 80 °C ist.

20. Beizverfahren nach Anspruch 11, wobei die abrasiven Partikel am Ende des Prozesses durch Filtration oder Absetzen zurückgewonnen werden.

## Revendications

1. Installation de décapage chimique destinée à appliquer un traitement de décapage chimique à une bande de métal (10) en un mouvement continu, ledit traitement de décapage chimique utilisant une solution acide, ladite installation de décapage chimique comprenant :
- une pluralité de cuves de traitement en cascade (1A, 1B, 1C, 1D, 1E, 1F, 11, 12, 13, etc.) parmi lesquelles au moins une cuve de traitement (1A, 1B, 1C) comprenant une section de pulvérisation/d'injection (3, 4, 7) destinée à pulvériser/injecter la solution acide sur la bande de métal (10), et
- des moyens de collecte (8, 9) destinés à récupérer la solution acide pulvérisée après utilisation et à rediriger celle-ci vers chaque section de pulvérisation/d'injection (3, 4, 7) ;
l'au moins une cuve de traitement (1A, 1B, 1C) comprenant un premier collecteur (2A) utilisé en face d'une première face de la bande de métal (10) et un deuxième collecteur (2B) utilisé en face d'une deuxième face de la bande de métal (10), **caractérisée en ce que** :
- dans une première configuration des cuves de traitement (1A), chacun du premier collecteur (2A) et du deuxième collecteur (2B) possède une surface plane interne (6) destinée à être respectivement parallèle à la première et à la deuxième faces de la bande de métal (10), et à une distance de celles-ci, en définissant un premier espace (5A) et un deuxième espace (5B) respectivement, ledit premier collecteur (2A) et ledit deuxième collecteur (2B) comprenant chacun une pluralité d'orifices (3) percés à travers la surface plane interne (6) selon un motif en 2D prédéfini, destinés à pulvériser la solution acide sur la bande de métal (10) en jets droits (4), dans des conditions adéquates pour créer, pendant l'utilisation, un coussin de liquide hautement turbulent (5') au niveau de la surface de la bande de métal (10), ou, en variante,
- dans une deuxième configuration des cuves de traitement (1B), chacun du premier collecteur (2A) et du deuxième collecteur (2B) possède une surface plane interne (6) destinée à être respectivement parallèle à la première et à la deuxième faces de la bande de métal (10), et à une distance de celles-ci, en définissant un premier espace (5A) et un deuxième espace (5B) respectivement, des moyens d'injection de solution acide étant prévus au niveau d'une ouverture d'injection de bord (7) de chaque espace respectif (5A, 5B) dans des conditions adéquates pour créer, pendant l'utilisation, une zone de liquide hautement turbulente occupant le volume total de l'espace respectif (5A, 5B) au niveau de la surface de la bande de métal (10) ou, en variante,
- une troisième configuration des cuves de traitement (1C) combine la première configuration des cuves de traitement (1A) et la deuxième configuration des cuves de traitement (1B) ;
et **en ce que**, soit dans la première configuration des cuves de traitement (1A), soit dans la deuxième configuration des cuves de traitement (1B), ladite surface plane interne (6) est continue, excepté aux endroits des orifices percés à l'intérieur dans le cas de la première configuration des cuves de traitement (1A).

2. Installation de décapage chimique selon la revendication 1, **caractérisée en ce que** la solution acide utilisée contient des particules abrasives.

3. Installation de décapage chimique selon la revendication 1 ou 2, **caractérisée en ce que** les moyens de collecte (8, 9) comprennent au moins une cuve de stockage (8) et au moins une pompe (9), ainsi qu'un moyen (18) destiné à injecter de l'acide neuf dans les cuves de décapage chimique à contre-courant par rapport au sens de mise en cascade.

4. Installation de décapage chimique selon la revendication 1 ou 2, **caractérisée en ce qu'**elle comprend au moins une autre cuve de traitement (11, 12, 13, ...).

5. Installation de décapage chimique selon la revendication 4, **caractérisée en ce que** l'au moins une autre cuve de traitement (11, 12, 13, ...) est une cuve de traitement par immersion ou rinçage.

6. Installation de décapage chimique selon la revendication 1 ou 2, **caractérisée en ce que** des guides latéraux sont prévus afin de maintenir le coussin de liquide (5') ou la zone hautement turbulente dans l'espace (5A, 5B), ou **en ce que** le premier et le deuxième espaces (5A, 5B) sont conçus pour former un tunnel ayant une largeur égale à la largeur de la ligne.

7. Installation de décapage chimique selon la revendication 3, **caractérisée en ce que** l'au moins une pompe (9) est composée d'un matériau capable de résister aux particules abrasives présentes à l'intérieur de la solution acide, choisi parmi le groupe constitué de la céramique, du graphite, du polyfluorure de vinylidène (PVDF) et du polytétrafluoroéthylène (PTFE).

8. Installation de décapage chimique selon la revendication 3, **caractérisée en ce que** l'au moins une pompe (9) est conçue de sorte que les particules abrasives soient injectées par effet Venturi après la sortie de la pompe.

9. Installation de décapage chimique selon la revendication 1 ou 2, **caractérisée en ce que** le premier espace (5A) et le deuxième espace (5B) sont différents.

10. Installation de décapage chimique selon la revendication 1 ou 2, **caractérisée en ce que** les moyens d'injection prévus au niveau d'une ouverture d'injection de bord (7) de l'espace (5A, 5B) sont à co-courant ou à contre-courant par rapport à la bande, dans ce dernier cas afin d'augmenter la vitesse relative entre la bande et le flux de décapage chimique.

11. Procédé d'application d'un traitement de décapage chimique à une bande de métal (10) en un mouvement continu, à l'aide de l'installation de décapage chimique selon l'une quelconque des revendications précédentes, **caractérisé en ce qu'**il comprend les étapes consistant à :
- alimenter l'installation de décapage chimique avec une solution acide ;
- diriger la bande de métal en mouvement (10) vers au moins une cuve de traitement (1A, 1B, 1C) comprenant une section de pulvérisation/d'injection (3, 4, 7) destinée à pulvériser/injecter la solution acide sur une ou sur les deux face(s) de la bande de métal (10) dans des conditions de forte turbulence ;
- récupérer la solution acide pulvérisée sur la bande de métal (10) et rediriger celle-ci vers les sections de pulvérisation/d'injection (3, 4, 7) à l'aide des moyens de collecte (8, 9).

12. Procédé de décapage chimique selon la revendication 11, **caractérisé en ce que** la bande de métal (10) est en outre dirigée dans une ou plusieurs autre(s) cuve(s) de traitement (11, 12, 13, ...) afin d'être traitée.

13. Procédé de décapage chimique selon la revendication 11, **caractérisé en ce que** la bande de métal (10) est une bande d'acier choisie parmi le groupe constitué de une bande d'acier au carbone, une bande d'acier inoxydable et une bande d'acier allié.

14. Procédé de décapage chimique selon la revendication 11, **caractérisé en ce que** la solution acide utilisée est une solution d'acide chlorhydrique, d'acide sulfurique, d'acide nitrique, d'acide phosphorique ou d'acide fluorhydrique.

15. Procédé de décapage chimique selon la revendication 11, **caractérisé en ce que** des particules minérales abrasives insolubles dans de l'acide (20) sont ajoutées à la solution acide.

16. Procédé de décapage chimique selon la revendication 15, **caractérisé en ce que** la dureté de Mohs des particules minérales abrasives insolubles dans de l'acide (20) est comprise entre 4 et 7.

17. Procédé de décapage chimique selon la revendication 15, **caractérisé en ce que** les particules minérales abrasives insolubles dans de l'acide (20) sont choisies parmi le groupe constitué du corindon, des microbilles de verre, de l'alumine, du silicate, du carbure de silicium et du zirconium.

18. Procédé de décapage chimique selon la revendication 11, **caractérisé en ce que** le débit de solution acide pulvérisée/injectée est choisi de façon à obtenir une épaisseur du coussin de liquide hautement turbulent (5') égale à l'épaisseur de l'espace (5) dans la première configuration de cuves (1A),.

19. Procédé de décapage chimique selon la revendication 11, **caractérisé en ce que** la température maximale de la solution acide est de 80°C, en cas d'utilisation de cuves en polypropylène, en PVDF ou en PTFE.

20. Procédé de décapage chimique selon la revendication 11, **caractérisé en ce que** les particules abrasives sont récupérées à la fin du processus par filtration ou décantation.
